

R. A. FESSENDEN.  
ARTIFICIAL LEATHER ARTICLE.  
APPLICATION FILED MAR. 15, 1920.

1,357,449.

Patented Nov. 2, 1920.



FIGURE 1



FIGURE 2



FIGURE 3



FIGURE 4

WITNESS:

Charles Myran  
Clair R. Myran

Reginald A. Fessenden.

INVENTOR.

# UNITED STATES PATENT OFFICE.

REGINALD A. FESSENDEN, OF CHESTNUT HILL, MASSACHUSETTS.

## ARTIFICIAL-LEATHER ARTICLE.

1,357,449.

Specification of Letters Patent.

Patented Nov. 2, 1920.

Application filed March 15, 1920. Serial No. 366,060.

To all whom it may concern:

Be it known that I, REGINALD A. FESSENDEN, of Chestnut Hill, in the county of Middlesex and State of Massachusetts, a citizen of the United States, have invented a new and useful improvement in Artificial-Leather Articles, of which the following is a specification.

My invention relates to methods and apparatus for making artificial leather and artificial leather articles, such as shoes, automobile coverings, and the like.

My invention has for its object improvement in the quality of such goods and more particularly improved methods and means for insuring adhesion between the artificial leather coating and the backing to which it is applied and means for making better joints between the different pieces of artificial leather composing the article and the preventing of the raveling of the edges of the pieces of artificial leather and in general producing a better article.

Figures 1, 2, 3, and 4 illustrate partly diagrammatically suitable methods and means for carrying out my invention.

Artificial leathers are, as a rule, formed by applying a coating of some material having the appearance of leather, generally a nitro-cellulose compound, to a backing of some fibrous material, generally cotton cloth or felt. One of the chief difficulties in producing durable articles of this type of artificial leather, such as shoes and similar articles, is lack of adhesion between the coating and the backing.

I overcome this difficulty by tufting, or quilting or stitching the fibrous backing in the manner shown in Fig. 1, where 13 is the backing of cotton cloth and 11, 11, 11, 11 are loops of thread, preferably cotton, and tufted at the end as shown.

When the coating 21 is applied to the outer surface of the backing 13 it engages 45 with the tufts and adheres thereto.

In order to insure still more complete adhesion of the backing I prefer to form the tufted or quilted material of a substance partly soluble in the coating. For example, 50 if the coating is a nitro-cellulose compound dissolved in a suitable solvent, I prefer to form the tufts 11, 11, 11, 11 or thread 12, 12 of nitrated cotton thread, which is stitched into the backing 13 and on the coating 21 being applied to the outer surface of

the backing 13, the tufts 11, 11 or thread 12, 12 partially dissolve and consequently a firm and integral union is made when the solvent dries out and the material hardens.

If desired the nitro-cellulose threads 11, 60 11 and 12, 12 may be denitrated from the back so that the inner portions of these threads are of denitrated material.

A second difficulty has been the fact that when shoes are made out of artificial leather 65 of the coated backing type the pieces of leather composing the shoe have been cut from a large piece of artificial leather, thereby leaving the edges of the backing exposed and liable to raveling of the backing and chipping off of the edges of the coating, thereby producing bad appearance and slipping of the stitching.

I overcome this by a new method—i. e. I first of all cut out pieces of backing of 70 the same shape that the pieces of artificial leather are formed when made up into the shoe and quilt the edges as shown at 19, Fig. 2, or stitch them as shown at 20, Fig. 2. I then load a large number of such pieces 75 on a moving table made of non-adhesive material, such as soapstone or slightly oiled brass, and apply the backing to all of these pieces, thereby producing leather parts 80 which are not liable to ravel or chip at the 85 edges.

I also prefer to quilt by tufts or threads of nitrated cotton such portions of the leather pieces as are liable to bending; for example as shown at 21, Fig. 2, across the 90 toe piece of the leather, 18 being the portion forming the toe, or to weave the backing with say twenty per cent. of nitrated threads.

A third difficulty which is met with is the 95 fact that even where the adhesion is good the coating, being less elastic than the backing, is liable to crack on bending, as shown in Fig. 3 where the backing 13 has been bent and the coating 21 has cracked as shown.

I overcome this by using a backing having two neutral axes, such for example as the material known as uncut double web cotton plush or velvet in which two pieces of velvet are woven together face to face, as shown in 100 Fig. 4 (the velvet being subsequently made by cutting down through the center).

I prefer to use this material, however, without its being cut down the center, as shown in Fig. 4 where 14 is one backing of 110

the velvet, 14' the other backing of the velvet, and 15 the velvet pile between the two backs.

On applying the coating 21 to the back 14, which in this case is the upper surface, it will be seen that when the backing is bent the coating 21 will not be stretched in the manner shown in Fig. 3 and will therefore remain adherent because one of the neutral axes, *i. e.* the neutral axis formed by the back 14, is directly adjacent to the coating 21.

I have found by experiment and test that this arrangement gives very good results and multiplies the life of the material many times.

The fourth difficulty is the making of suitable joints between the different pieces of leather forming the shoe. I have found that 20 using uncut double web cotton plush or velvet overcomes this difficulty, since if the edges be quilted as shown at 16, Fig. 4, or stitched, as shown at 17, Fig. 4, the edges are compressed as shown so that when two 25 pieces are laid side by side and stitched together the joint may be made substantially smooth, due to the compression of the pile and the subsequent diminution of thickness at the edge.

30 By these means I am able to produce a satisfactory artificial leather shoe and satisfactory articles of similar character.

After coating, the pieces of artificial leather are preferably pierced by numerous

minute needles so as to provide for satisfactory ventilation and the inner side of the backing is preferably treated with boracic acid or similar antiseptic material.

What I claim as my invention is:—

1. An artificial leather comprising a coating and a backing and stitches inserted in the backing and in contact with the coating, such stitches being formed of a material uniting integrally with the coating.

2. An artificial leather comprising a soluble coating and a backing and stitches inserted in the backing and in contact with the coating, said stitches being soluble in the solvent of the coating.

3. The method of making shoes from artificial leather comprising a coating and a backing which consists in first cutting the backing to shape, then stitching it around the edges, and then applying the coating, whereby the piece of artificial leather is prevented from raveling and chipping at the edges.

4. An artificial leather comprising a coating and a backing, said backing consisting of a material having two neutral axes filamentarily connected so as to be relatively shiftable, said coating being applied to one of said neutral axes.

5. An artificial leather comprising a soluble coating and a backing, said backing containing a small percentage of threads of a material soluble in the solvent of the coating.

REGINALD A. FESSENDEN.